

Patented Mar. 21, 1933

1,902,539

# UNITED STATES PATENT OFFICE

CARL FRIEDRICH BRAUER, OF STETTIN, GERMANY

## STENCIL

No Drawing. Application filed April 16, 1931, Serial No. 530,723, and in Germany October 28, 1930.

This invention relates to stencil sheets adapted for the reproduction of written and typewritten matter.

Stencil sheets have been made generally from a base sheet of open texture, fibrous paper provided with a coating that is impervious to ink, but which may be cut on a typewriter or with a stylus to permit the passage of ink for reproduction of copies. The paper base commonly used is that known in the art as Yoshino. Although various kinds of coating materials have been used, all of the stencils heretofore commercially available have been subject to certain disadvantages.

The first stencils had a coating of wax. Such coatings are readily cracked and broken, which permits the ink to penetrate the stencil and spoil the copies, and they are affected adversely by varying climatic conditions. The wax stencils were largely superseded by those having a coating of gelatin coagulated, or hardened, by a chromium salt, formaldehyde, or the like agent. These tanned gelatin stencils are very strong and have a long useful life, but they must be moistened to render the coating type-impermeable. This is disadvantageous because the liquid used for moistening the stencils causes rusting and corrosion of typewriter parts. Also, the sheets stretch when moistened, and therefore the material to be reproduced may become distorted either during cutting of the wet stencil, or during its drying. The coagulated gelation stencils furthermore have had considerable tendency to form pin holes in the coating which permit ink to seep through and spot the copies made from them.

More recently there have been developed the so-called dry stencils, whose coating comprises a cellulose compound, such as cellulose nitrate, softened and rendered type impermeable by oils. Such cellulose dry stencils do not require moistening, and they are satisfactorily strong at first. But the oils tend to sweat out, and this impairs the keeping qualities of the stencils and causes damage to the rubber parts of the typewriter which come in contact with them.

It is among the objects of this invention to provide stencil sheets having a coating which is type-impermeable without moistening or otherwise treating it before being cut, is strong, free from pinholes, and not subject to cracking, produces clean and sharp copies, may be made from a composition that is simple and readily prepared and used, and which overcomes or minimizes the disadvantages of prior stencil sheets.

The invention is predicated upon my discovery that satisfactory stencil sheets embodying the objects stated may be prepared from gelatin without hardening or coagulating it. In accordance with the invention this is accomplished by coating or impregnating an open texture, fibrous base, such as Yoshino, with a composition adapted to form a coating of non-coagulated gelatin having homogeneously dispersed therethrough an oily softening agent and a stabilizing material. As used herein the terms "stabilizer" and "stabilizing material" have reference to substances which do not coagulate the gelatin but maintain the coating supple and homogeneous, and prevent sweating out of its ingredients. The coating thus provided can be cut with type or stylus without moistening, and is therefore directly stencilizable.

In the practice of this invention the coating composition is made by swelling, or dissolving, a gelatin having suitable strength. Water may be used for this purpose, but it is preferred to amplify the swelling due to water by means of an acid. Acetic acid is preferred for this purpose because it effects an even and uniform swelling and distribution of the gelatin in the coating composition. The acid appears also to dissolve the gelatin somewhat, and this is helpful in obtaining a homogeneously dispersed composition. To the gelatin solution there is added a softening agent in an amount sufficient to render the gelatin in the coating soft and type-impermeable. Oleic acid may be, and preferably is, used for this purpose. The composition preferably includes also a fixed solvent, such as Turkey red oil, which also has oily characteristics. The Turkey red

55

60

65

70

75

80

85

90

95

100

oil preferably is used with another solvent, such as alcohol.

Stencil sheets prepared from a composition containing the materials just described are stencilizable to give satisfactory results. However, they have a tendency to exude a certain amount of the oil incorporated in the coating solution, and they harden and become brittle. This reduces the impressibility of the coating and leakage of ink through the cracks soils the copy paper.

The invention is predicated in part upon my discovery that these disadvantages may be overcome and fully satisfactory stencil sheets produced by incorporating with the coating composition a material adapted to maintain the ingredients in the coating in a homogeneous stable condition. Such materials are herein termed stabilizers. I have discovered that the higher chlorinated naphthalenes are particularly suitable for this purpose, and especially the hexachlorinated naphthalenes. I now believe the beneficial action to be due to formation of a solid solution with the oleic acid. Be that as it may, the stabilizers maintain the coatings homogeneous and stencilizable, and they minimize the disadvantages of unhardened gelatin coatings not containing them.

These chlorinated naphthalenes can be dispersed readily in a solution containing alcohol or Turkey red oil. Other stabilizers may be used instead of the chlorinated naphthalenes referred to; e.g., either palmitic or stearic acids, both of which are stabilizers, may be used, in which case the palmitic or stearic acid replaces a portion of the oleic acid. Compositions containing these stabilizers have excellent coating qualities, and they provide stencil sheets having a coating that does not exude its ingredients, does not become brittle, and remains homogeneous. The sheets produce clear and clean copies, and, because the stabilizers do not irreversibly harden, or coagulate the gelatine, they are ready for immediate use, i.e. they are directly stencilizable.

There may be added also to the composition a small amount of a cellulose ester, such as cellulose nitrate. This also tends to maintain the homogeneity of the coating and improve the cutting qualities of the sheet. For this purpose the cellulose ester may be incorporated in the oleic acid, or dissolved in a solvent such as butyl acetate. In this connection it is to be observed that the cellulose ester represents a preferred addition, and when so used constitutes a minor proportion only of the coating.

In the preferred practice of the invention one part of powdered gelatin is mixed with ten parts of water. After the gelatin has begun to swell there is added acetic acid equivalent to 6 per cent of glacial acid calculated upon the dry weight of the gelatin.

The mixture is allowed to stand at room, or slightly above room, temperature until it has become thick and highly viscous and will remain so at room temperature.

There is prepared also a second solution comprising about one and one-half parts of hexachlornaphthalene and two parts of oleic acid, both calculated upon the dry gelatin weight. These ingredients are dissolved in double the quantity of a solution of equal parts of alcohol and Turkey red oil. This second solution is quite clear and transparent. The coating composition is then made by mixing two parts of the latter solution with one part of the thick gelatin solution, the mixture being vigorously agitated or stirred until a perfectly homogenous dispersion has been obtained.

In case it is desired to use the cellulose ester referred to hereinabove, there may be added to the solution of hexachlornaphthalene and oleic acid about 0.5 per cent (calculated upon the total of the final mixture) of cellulose nitrate in the form of a solution in butyl acetate. The mixture of oleic acid, hexachlornaphthalene and cellulose nitrate is then added to the gelatin solution in the proportions just described.

Stencil sheets are made by drawing Yoshino paper through or over the composition, the excess composition being removed, and the sheets dried. This procedure is well known in the art and requires no further detailed description. During coating of the sheets it is advisable to warm the coating composition somewhat so as to reduce its consistency and prevent it from getting too thick. When the sheets are drawn the coating mass is milky in appearance, but after having dried it becomes transparent, uniform and readily stencilizable. It will be understood that colored coatings may be provided by dissolving a dye in the composition, or suspending a colored pigment in it.

According to the provisions of the patent statutes, I have explained the principle of my invention, and have described what I now consider to represent its best embodiment. However, I desire to have it understood that, within the scope of the appended claims, the invention may be practiced otherwise than as specifically described.

I claim as my invention:

1. A directly stencilizable stencil sheet comprising an open texture fibrous base coated with a composition including gelatin highly distended in an aqueous solution of acetic acid and having homogeneously dispersed therethrough oleic acid and a non-coagulating stabilizer of the group comprising chlorinated naphthalene, palmitic acid and stearic acid, the gelatin in the coated sheet being in an unhardened and uncoagulated condition, and said stabilizer

maintaining the homogeneity and permanence of the coating.

2. A directly stencilizable stencil sheet comprising an open texture fibrous base having a coating of gelatin in an unhardened and uncoagulated highly distended condition, the gelatin having homogeneously dispersed therethrough oleic acid and chlorinated naphthalene, the chlorinated naphthalene being present in an amount less than the oleic acid, and said oleic acid rendering the coating supple, and said chlorinated naphthalene maintaining the homogeneity and permanence of the coating.

15 3. A directly stencilizable stencil sheet comprising an open texture fibrous base having a coating of gelatin in an unhardened and uncoagulated highly distended condition, the gelatin having homogeneously dispersed therethrough a solid solution of a major proportion of oleic acid and a minor proportion of a non-coagulating stabilizer of the group comprising chlorinated naphthalene, palmitic acid and stearic acid, said oleic acid rendering the coating supple, and said stabilizer maintaining the homogeneity and permanence of the coating.

4. A directly stencilizable stencil sheet comprising an open texture fibrous base having a coating of gelatin in an unhardened and uncoagulated highly distended condition, the gelatin having homogeneously dispersed therethrough oleic acid, a non-coagulating stabilizer of the group comprising chlorinated naphthalene, palmitic acid and stearic acid, and also containing a minor proportion of a cellulose ester, the homogeneity and permanence of the coating being maintained by said stabilizer and ester.

45 5. A directly stencilizable stencil sheet comprising an open texture fibrous base having a coating of gelatin in an unhardened and uncoagulated highly distended condition, the gelatin having homogeneously dispersed therethrough a solid solution of oleic acid and a non-coagulating stabilizer of the group comprising chlorinated naphthalene, palmitic acid and stearic acid, said stabilizer being present in an amount less than the oleic acid, and a minor proportion of a cellulose ester, the homogeneity and permanence of the coating being maintained by said stabilizer and ester.

55 6. A directly stencilizable stencil sheet comprising an open texture fibrous base having a coating of gelatin in an unhardened and uncoagulated highly distended condition, the gelatin having homogeneously dispersed therethrough oleic acid, a non-coagulating stabilizer of the group comprising chlorinated naphthalene, palmitic acid and stearic acid, said stabilizer being present in an amount less than the oleic acid, a minor proportion of a cellulose ester,

and Turkey red oil, the homogeneity and permanence of the coating being maintained by said stabilizer and ester.

7. A process of making a directly stencilizable stencil sheet, comprising coating an open texture fibrous base with a coating composition of gelatin, aqueous acetic acid, oleic acid, and a non-coagulating stabilizer of the group comprising chlorinated naphthalene, palmitic acid and stearic acid, said acetic acid rendering the gelatin highly absorptive of said oleic acid and stabilizer, the gelatin in the coated sheet being in an unhardened and uncoagulated condition, and said stabilizer maintaining the homogeneity and permanence of the coating.

8. A process of making a directly stencilizable stencil sheet comprising coating an open texture fibrous base with a coating composition of gelatin, aqueous acetic acid, oleic acid, a stabilizer in an amount less than said oleic acid and selected from the group comprising chlorinated naphthalene, palmitic acid and stearic acid, and a minor proportion of cellulose ester, said acetic acid rendering the gelatin highly absorptive of the remaining ingredients, the gelatin in the coated sheet being in an unhardened and uncoagulated condition, and the homogeneity and permanence of the coating being maintained by said stabilizer and cellulose ester.

9. A directly stencilizable stencil sheet comprising an open texture fibrous base having a coating of gelatin in an unhardened and uncoagulated highly distended condition, the gelatin having homogeneously dispersed therethrough Turkey red oil and a solid solution of a major proportion of oleic acid and a minor proportion of a non-coagulating stabilizer of the group comprising chlorinated naphthalene, palmitic acid, and stearic acid, said oleic acid rendering the coating supple, and said stabilizer maintaining the homogeneity and permanence of the coating.

10. A process of making a directly stencilizable stencil sheet comprising coating an open texture fibrous base with a coating composition of gelatin, aqueous acetic acid, Turkey red oil, oleic acid, a stabilizer in an amount less than said oleic acid and selected from the group comprising chlorinated naphthalene, palmitic acid and stearic acid, a minor proportion of cellulose ester, said acetic acid rendering the gelatin highly absorptive of the remaining ingredients, the gelatin in the coated sheet being in an unhardened and uncoagulated condition, and the homogeneity and permanence of the coating being maintained by said stabilizer and cellulose ester.

In testimony whereof, I hereunto sign my name.

CARL FRIEDRICH BRAUER. 130